

Patented Feb. 1, 1949

2,460,400

# UNITED STATES PATENT OFFICE

2,460,400

## METHODS FOR THE TREATMENT OF REGENERATED CELLULOSE THREAD

Carl Schlatter, Wilmington, Del., and Carl V. Holmberg, Crossett, Ark., assignors to American Viscose Corporation, Wilmington, Del., a corporation of Delaware

No Drawing. Application July 13, 1944,  
Serial No. 544,824

4 Claims. (Cl. 117—139.5)

1

This invention relates to methods of treating moisture-laden filamentary material, particularly in conjunction with the manufacture of artificial filaments. More particularly, the invention relates to methods of treating moisture-laden filamentary material in the form of wound packages for the purpose of drying and/or conditioning them.

The procedure of our invention is applicable to moisture-laden filamentary material of all types, but for purposes of illustration will be discussed here more particularly as used in connection with artificial filamentary material produced in accordance with the viscose process. According to that process, the spinning dope is extruded into a suitable aqueous coagulating medium, and the thread or yarn thus obtained is collected on a perforated tube, in bobbin spinning, or in a rotating centrifuge or spinning bucket in the form of a package constituted by a thread wound upon itself in a plurality of layers and known as a rayon "cake." Such packages or cakes are then subjected to a number of after-treatments in aqueous liquids, such as bleaching, desulfurizing, and washing, and are then dried while still in package form.

The conventional drying procedure involves centrifuging the cakes to remove excess surface moisture, followed by exposure thereof to the action of warm air currents circulated mainly around the packages. Unless that drying procedure is carried out very slowly, under carefully controlled temperature and humidity conditions, it results in very undesirable differences in yarn properties throughout the yarn package, which differences are most marked in the case of elongation, residual shrinkage capacities, and dyeing affinities. Such differences are mostly due to the fact that the various portions of the yarn package are not subjected to the same drying conditions and therefore do not dry uniformly. The outer convolutions tend to dry before the inner convolutions, and because of this difference in drying rate, the outer convolutions cannot shrink during drying, so that stresses and strains are set up in the outer windings of the package, resulting in what is herein termed "case-hardening" and the development of non-uniform dyeing affinities and physical properties along the entire length of the filamentary material comprising the package.

It has also been proposed to dehydrate moisture-laden filamentary material by displacing the water by means of an organic solvent such as

2

ethyl alcohol, hydrocarbons such as paraffin oil, solvent naphtha, etc. However, those methods of dehydration are unsatisfactory in a number of important respects which renders them entirely unsuitable for dehydration of filamentary material particularly on a large-scale commercial basis. In the case of alcohol, for example, the costs are excessive and it has been found that when wound packages of filamentary material are treated with alcohol, it is impossible to remove all of the adhering alcohol therefrom by centrifuging at least 15 to 20% thereof remaining in the package which is only gradually evaporated off over a more or less extended period of time which represents a loss of the alcohol or requires a solvent recovery system which adds considerably to the expense of manufacturing the filamentary material.

The use of hydrocarbon solvents, such as solvent naphtha or the like for dehydrating filamentary material is disadvantageous for the reason that such solvents are naturally very hydrophobic and the water-withdrawing capacity thereof is extremely low. If it is desired to effectively dehydrate moisture-laden filamentary material, and particularly wound packages of such material, by means of hydrocarbon solvents, such as solvent naphtha, benzene, toluene, etc., it is necessary to subject the material to innumerable repetitive treatments with fresh solvent over prolonged periods and at temperatures of 80 to 100° C., which results in degradation of material, especially in the case of rayon, so that the final dried product is not suitable for the production of knitted, woven, or otherwise fabricated articles of good quality.

It is an object of the present invention to provide a method of drying filamentary material which does not involve the disadvantages of known methods and which yields a final product of superior quality. It is a further object of the invention to provide a method of drying which greatly reduces the period of drying time. Still another object of the invention is to provide a method for simultaneously drying filamentary material and applying a conditioning agent to the same so that it is made more amenable to textile processing. Other objects and advantages will appear hereinafter.

The disadvantages inherent in the known methods of drying are eliminated by the practice of the present invention, according to which it has been discovered that the water contained in

moisture-laden filamentary material is rapidly withdrawn therefrom in large amounts when volatile hydrocarbon solvents are applied thereto in conjunction with comparatively small amounts of an auxiliary water-withdrawing and blending agent which contains both hydrophilic and hydrophobic groups which are so balanced that the auxiliary agent is soluble in the hydrocarbon solvent and is capable of blending a substantial amount of water with the solvent into a single phase system having enduring stability. Such auxiliary water-withdrawing and blending agents must be sufficiently hydrophobic to be freely soluble in the hydrocarbon solvent and at the same time sufficiently hydrophilic to definitely attract water and to be appreciably soluble therein.

We have discovered that there are a number of substances which meet those requirements and which are capable of markedly enhancing the water-withdrawing capacity of volatile hydrocarbon solvents when applied in conjunction therewith. The agents contain at least one hydrophobic group, such as an aliphatic hydrocarbon group having at least 4 carbon atoms in a straight chain, in combination with hydrophilic groups, such as free hydroxyl groups, ether groups, and ester groups. The hydrophilic character may be the combined result of two or more such groups or it may be the result merely of one such group, but in any event, the hydrophilic content in any given compound is so balanced with respect to the hydrophobic content therein that the compound remains soluble in the volatile hydrocarbon solvent and the solution of it in such solvent can absorb a substantial amount of water without causing a separation into two or more distinct phases. An example of a highly satisfactory agent for use with solvent naphtha is the condensation product of ethylene oxide with stearic acid containing 10 ethylene oxide units per molecule. The related compounds may also be used. For example such a condensate containing 20 ethylene oxide units per molecule can be used but since it is not as soluble in the hydrocarbon as the 10-unit condensate, it cannot blend as high a percentage of water and is therefore not quite as efficient. However, such a condensate containing 40 ethylene oxide units per molecule is too hydrophilic since it is insoluble in the solvent naphtha. At the other extreme, a condensate with stearic acid containing only 5 ethylene oxide units per molecule is of reduced efficiency because of reduced water-withdrawing and blending capacity. Representative hydrophobic-hydrophilic substances which may be combined with the hydrocarbon solvents are the ethers or esters of polyhydric alcohols, and especially the partial ethers and esters which contain one or more free hydroxyl groups, including such partial ethers as Butyl Cellosolve, and partial esters of such polyhydric alcohols as sorbitol, mannitol, glycol, glycerol, etc., with fatty acids such as stearic, oleic, palmitic, myristic, lauric, etc. Representative specific compounds are the distearate of a polyethylene glycol containing 20 ethylene oxide units, also

Glycerol monopalmitate  
Glycerol monostearate  
Diethylene glycol mono-oleate  
Ethylene glycol mono-oleate  
Diethylene glycol mono-stearate  
Sorbitol distearate  
Sorbitol tri-stearate  
Sorbitol tetra-stearate

or any other partial esters of the alcohols. All of the esters listed may contain ethylene oxide groups, and the number of such groups present may vary within wide limits. Such compounds as sorbitol mono-, di-, tri-, or tetra-stearate containing six ethylene oxide groups, as well as substances of the type of polyethylene glycol monostearate containing ten ethylene oxide groups have been found effective. Esters from mixed fatty acids such as are obtainable from fish oils, vegetable oils, or animal fats, which may or may not be hydrogenated, may likewise be used. The esters may be in their pure state or in the form of their technical grades available on the market and in that form they vary from liquid oily, or pasty or firm waxy masses which generally are readily meltable at temperatures slightly above room temperature. They are substantially neutral and do not exhibit any swelling or other untoward effect on the filamentary material.

The hydrocarbon solvents and oleaginous water-withdrawing and blending agents form clear mixtures which exist as a continuous single phase system. The mixtures do not lose their clarity or become of emulsion or suspension type even when they are passed through the yarn packages and after the water has been withdrawn from the packages and blended therewith.

According to the invention one or more auxiliary water-withdrawing and blending agents of the type aforesaid may be added to a volatile hydrocarbon solvent of the paraffinic, naphthenic or aromatic series, including such solvents of the dry cleaning type derived from natural sources as Stoddard's solvent, the naphthenes or cycloparaffins, aromatic hydrocarbons such as benzene, toluene, solvent naphtha, the xylenes, or similar solvents. The hydrocarbons are solvents for the auxiliary water-withdrawing and blending agents, are normally immiscible with water but capable of being blended therewith in the presence of the auxiliary agent and do not adversely affect the filamentary material. To form the dehydration medium, the auxiliary blending agent may be added to the hydrocarbon solvent in any suitable amount, comparatively small quantities in the neighborhood of about 1 to 10% by weight being satisfactory, and depending upon the particular blending agent or agents selected, some improvement in efficiency may be noticeable at the higher concentrations. The temperature at which dehydration is effected may vary from about room temperature to around 100° C., temperatures in the neighborhood of about 80° C. having been found to be good practical working temperatures in most cases. The temperature should not be as high as or above the boiling point of water or the dehydration medium under the conditions of application.

The dehydration process may be carried out in any suitable manner. In the case of rayon cakes or other wound packages, it is advantageous to support the packages on a perforated pipe or tube and to pump the dehydrating solution or dispersion therethrough so that the same is forced through the package from the inside to the outside thereof. In this manner, dehydration of the packages proceeds uniformly, essentially from the inside of the packages, so that opportunity for the development of internal strains in the package does not occur and all of the layers constituting the various strata of the package are dried at substantially the same rapid rate and under practically the same temperature conditions. The amount of water withdrawn may be

controlled, and dehydration may be so effected that the packages or cakes retain substantially the moisture content normally desired in commercial grades of filamentary material which, in the case of regenerated cellulose, for example, is about 11%, or the method may be applied in connection with procedures in which the removal of the moisture is effected in separate stages of a multiple stage process. In some instances, it may be preferred to partially dehydrate the package by means of comparatively small amounts of the hydrocarbon solvent-blending agent medium and then complete the drying of the package by other methods. After completion of the treatment of the packages with the dehydrating solution, any surplus dehydrating medium remaining with the package may be removed by centrifuging and then the small amount remaining (approximately 10% for hydrocarbon solvents) is left to evaporate and as such solvents are inexpensive this is no economic handicap. Also such evaporation causes no "case hardening" and all parts of the cake are uniformly dried and of uniform quality.

The application of a dehydrating solution in accordance with the instant invention to moisture-laden wound packages of filamentary material results in a striking improvement in the rate and amount of water withdrawn therefrom, and a consequent marked reduction in drying time, the solution having the capacity of withdrawing water in the amount of 10,000 to 100,000 or more parts of water to a million parts thereof, as contrasted to two parts of water withdrawn by a million parts of hydrocarbon solvent when the latter only is applied to the filamentary material under comparable temperature conditions. It has been determined by repeated experiment that, whereas drying methods involving the circulation of warm air currents require at least three days, and the use of hydrocarbon solvents alone requires about the same time or longer, in the present case the packages are satisfactorily dried in a matter of about three hours or less depending on the speed of circulation of the medium.

The dehydrating medium may be applied to moisture-laden filamentary material in a form other than a wound package as for example to fibers in the form of a tow, felt or fabric, or to running lengths thereof, the fibers or articles comprising the same being continuously drawn through a path along which they come into contact with the medium which may be sprayed on or otherwise applied thereto.

Preferably, after the dehydrating medium has been passed through the wound package or applied to fibers in other forms, it is recycled and water evaporated therefrom in order to maintain its dehydrating efficiency.

During the dehydrating process some of the water is displaced by the oleaginous water-withdrawing and blending agent so that the latter remains firmly fixed upon the material, and the process may be so effected that lesser or greater amounts of the blending agent remain with the yarn or the like. Since the preferred blending agents are of the lubricating type of substance which is frequently applied to filamentary material preparatory to textile processing thereof, for example, to render the same more easily manipulable in knitting and weaving operations, that is to facilitate passage of the filaments through the knitting or weaving machines, the presence of the blending agent on the material is not objectionable and may be highly desirable and intentional. Thus, our invention may be regarded

as a combination simultaneous dehydrating and conditioning operation in which the conditioning agent is applied to the filamentary material while the latter is in the moist condition. The amount of conditioning or lubricating agent, i. e. of an auxiliary water-withdrawing and blending agent of oleaginous character or of waxy character where it is desired to size or set the twist of yarns or fabrics remaining on the filamentary material after withdrawal of the water therefrom may be predetermined and varied within fairly wide limits by controlling the temperature at which the dehydrating process is carried out, the particular oleaginous or waxy water-withdrawing and blending agent selected, and the concentration thereof employed, so that a wide latitude in these conditions is possible and permissible for obtaining special results. Although the oleaginous or waxy water-withdrawing and blending agent is hydrophobic to some extent, it is sufficiently hydrophilic to permit of its being removed from fabrics made from the treated filamentary material by ordinary scouring methods. As examples of our invention, when a dehydrating medium consisting of Stoddard's solvent and 5% by weight of sorbitol distearate containing six ethylene oxide groups was passed from the inside through all parts of moist rayon cakes at 80° C., about 8 to 10% of the sorbitol distearate compound remained on the material after withdrawal of the water therefrom. On the other hand, after the water was withdrawn from moist cakes by passing therethrough a medium consisting of Stoddard's solvent and 5% by weight of polyethylene glycol distearate containing twenty ethylene oxide groups, at 70° C., 1% of the distearate remained on the dehydrated cakes.

This method of simultaneously dehydrating filamentary material and applying a textile conditioning agent thereto has many important advantages when applied to rayon cakes or other wound packages since it facilitates even and thorough penetration of the conditioning agent throughout all strata of the package, the agent taking the place of withdrawn water, and there is no tendency for the conditioning agent to migrate from one stratum of the package to another upon the final removal of excess dehydrating medium, such as is often experienced when lubricating or other conditioning agents are applied to wound packages of filamentary material from simple solutions thereof in aqueous or organic solvents. This appears to be the result of a definite partitioning ratio between the filamentary material and the blended dehydrating medium-water solution.

A striking feature of the present invention resides in the fact that the dried product obtained by means of our new dehydrating procedure is of decidedly different and vastly superior quality as compared with filamentary material dried by other methods, being characterized by greater softness and pliability and an improved fluffy handle or feel, which is obtained without any impairment in elongation, tensile strength, or other desirable physical property. This marked superiority of the dried material as to softness and increased workability apparently results from the use of the auxiliary water-withdrawing and blending agent in the dehydration procedure, but is not due merely to the presence thereof on the dried material, since the improvement is observed, regardless of the amount thereof remaining on the material, and even when only minute amounts are present. A dried product of

the same or comparable quality cannot be obtained by any other known drying method, and is not obtained when filamentary material which has been previously dried by such known methods is subsequently impregnated with a lubricant or conditioning agent in a separate operation.

To illustrate one method of practicing our invention, cakes comprising freshly spun viscose rayon coming directly from the last washing stage of the after-treatment stages of the viscose rayon process, including bleaching, desulfurizing, and washing were centrifuged to remove excess surface water, after which they contained about 150 to 200% of water. A solution consisting of Stoddard's solvent and 5% of sorbitol distearate containing six ethylene oxide groups, at 80° C., was then passed through the cakes from the inside to the outside thereof. After three hours, the cakes were centrifuged and the water content was found to have been reduced to about 10% on a bone-dry basis, and about 10% of the sorbitol distearate compound remained on the filamentary material.

Instead of the dehydrating medium employed above, a solution consisting of any other similar partial ester of a polyhydric alcohol, or partial ether thereof, and any other hydrocarbon or chlorinated hydrocarbon solvent may be employed.

While the invention is particularly suitable for the initial dehydration of freshly produced regenerated cellulose rayon in wound package form, it is not limited thereto, and may be applied with similar noteworthy results to other textile materials such as yarns of cotton, wool, real silk, cellulose acetate, or other natural or artificial fibers.

From the foregoing discussion, it will be apparent that we have devised an entirely new method of rapidly dehydrating and conditioning moisture-laden filamentary material by means of which it is possible to utilize the readily available and cheap hydrocarbon or chlorinated hydrocarbon dry-cleaning solvents modified by the incorporation therewith of only relatively small amounts of auxiliary water-withdrawing and blending agents. The process is simple, extremely economical, and yields a dried product which is of high quality, characterized by uniform tensile strengths, residual shrinkage capacities, and dyeing affinities throughout and which is suitable for working into knitted, woven or otherwise constructed fabrics of uniformly good quality. The fact that the process may be so practiced as to result in the simultaneous dehydration and conditioning of the filamentary material to any desired extent is of special consideration in some cases, since it eliminates the necessity for subjecting the material to separate lubricating, sizing, twist-setting, or other conditioning procedures in those instances where the presence of the conditioning agents in appreciable amounts is desired or necessary.

While preferred embodiments of the invention have been described, the description herein is intended to be illustrative only, and it is to be understood that changes and variations may be made without departing from the spirit or scope of the invention as defined by the appended claims.

We claim:

1. In the method of manufacturing artificial filaments of regenerated cellulose from viscose comprising spinning the filament-forming material into an aqueous coagulating medium and

subjecting the filaments to aqueous after-treatment, including final washing, the step of continuously over a predetermined interval of time treating the filaments while still wet from the washing step and before any prior drying thereof, with a solution comprising a volatile hydrophobic hydrocarbon solvent and from about 1 to 10% of an organic compound capable of withdrawing water from the filamentary material and blending the withdrawn water with the hydrocarbon solvent into a substantially single phase system, said organic compound being soluble in the hydrocarbon solvent, containing at least one hydrophobic group and at least one hydrophilic group, and comprising a substance selected from the group consisting of partial esters of polyhydric alcohols with fatty acids having from 12 to 18 carbon atoms, and ethylene oxide condensates of such esters containing from 6 to 20 ethylene oxide units, such treatment being performed at a temperature below the boiling points of water and the solvent under the conditions of application, and continuously removing the resulting blended system from the filamentary material thereby leaving the material in a predetermined state of dryness.

2. In a method of manufacturing regenerated cellulose thread from viscose, the step of treating a moisture-laden wound package of the thread, after washing thereof as a stage in its manufacture and before any prior drying thereof, which comprises continuously passing through all parts of the package a solution comprising a hydrocarbon dry-cleaning solvent and from about 1 to 10% by weight of a sorbitol partial stearate containing six ethylene oxide groups, and continuously removing water carried by the thread in a blended, single phase system with the hydrocarbon dry cleaning solvent and polyhydric alcohol derivative.

3. In a method of manufacturing regenerated cellulose thread from viscose, the step of treating a moisture-laden wound package of the thread, after washing thereof as a stage in its manufacture and before any prior drying thereof, which comprises continuously passing through all parts of the package a solution comprising Stoddard's solvent and 5% by weight of sorbitol distearate containing six ethylene oxide groups, said treatment being performed at a temperature of about 80° C., and continuously removing water carried by the thread in a blended, single phase system with the hydrocarbon dry cleaning solvent and polyhydric alcohol derivative.

4. In a method of manufacturing regenerated cellulose thread from viscose, the step of treating a moisture-laden wound package of the thread, after washing thereof as a stage in its manufacture and before any prior drying thereof, which comprises continuously passing through all parts of the package a solution comprising Stoddard's solvent and 5% by weight of polyethylene glycol distearate containing twenty ethylene oxide groups, said treatment being performed at a temperature of about 70° C., and continuously removing water carried by the thread in a blended, single phase system with the hydrocarbon dry cleaning solvent and polyhydric alcohol derivative.

CARL SCHLATTER.  
CARL V. HOLMBERG.

(References on following page)

## REFERENCES CITED

The following references are of record in the file of this patent:

## UNITED STATES PATENTS

| Number    | Name             | Date          |
|-----------|------------------|---------------|
| 1,945,959 | Williams         | Feb. 6, 1934  |
| 1,959,930 | Schmidt et al.   | May 22, 1934  |
| 1,970,578 | Schoeller et al. | Aug. 21, 1934 |
| 1,999,585 | Buggeman         | Apr. 30, 1935 |

| Number    |
|-----------|
| 2,017,177 |
| 2,119,117 |
| 2,127,586 |
| 2,137,404 |
| 2,273,636 |
| 2,275,494 |
| 2,297,135 |
| 2,380,166 |
| 2,418,752 |

| Name              | Date           |
|-------------------|----------------|
| Bassett           | Oct. 15, 1935  |
| Schuller          | May 31, 1938   |
| Dreyfus           | Aug. 23, 1938  |
| Hollerer          | Nov. 22, 1938  |
| Gellendien et al. | Feb. 17, 1942  |
| Bennett           | Mar. 10, 1942  |
| Davis et al.      | Sept. 29, 1942 |
| Griffin           | July 10, 1945  |
| Brown             | Aug. 8, 1947   |